# EUROPEAN PATENT SPECIFICATION

(11) **EP 1 993 109 B1**
(45) Date of publication and mention of the grant of the patent: **04.06.2014**
(21) Application number: 07108466.9
(22) Date of filing: 18.05.2007
(51) Int. Cl.: H01C 7/12, H01C 7/10, H01C 7/105

(54) **Surge absorbing material with a further electrical function**
Material zur Absorption von elektrischen Störimpulsen mit einer weiteren elektrischen Funktion
Matériel absorbant des impulsions parasites avec une fonction électrique supplémentaire

(43) Date of publication of application: 19.11.2008
(73) Proprietor: SFI Electronics Technology Inc., Taiwan (CN)
(72) Inventor: Tan, Yu-Wen, c/o Leader Well Technology Co., Ltd., Guishan Shiang, Taoyuan County 333 (TW); Zhu, Jie-An, c/o Leader Well Technology Co., Ltd., Guishan Shiang, Taoyuan County 333 (TW); Zhang, Li-Yun, c/o Leader Well Technology Co., Ltd., Guishan Shiang, Taoyuan County 333 (TW)
(74) Representative: Beck, Michael Rudolf

(56) References cited:
- EP-A- 1 585 146
- WO-A-88/00526
- KR-A- 20020 028 279

## Description

### BACKGROUND OF THE INVENTION

### 1. Field of the Invention

The present invention relates to a surge absorbing material.

### 2. Description of the Related Art

Surge or electrical overstress produced by a lightning strike, switching operation or damage of other component may disturb or damage electronic components or other sensitive electric equipment. Therefore, surge absorbers (or called varistors) with good surge absorbing capability are widely used as components for providing protection against electrical overstress or surge of electronic components, electronic circuits or electronic equipment.

Moreover, it is a popular trend to combine two components of different functions as a single structure by a laminating process. For example, inductance and capacitance are combined as a single SMD-type (surface mounting device) component to become an inductance-capacitance filter (LC filter) with filtering function; or, resistance and capacitance are combined as a single SMD-type component to become a resistance-capacitance filter (RC filter) with filtering function.

However, when two components of different functions are combined as a single structure by a laminating process, a residual stress is easily occurred between the two components because sintering temperatures and shrinkage rates of the two components are different, and then there are problems of separation and ineffectiveness occurred after the two components of different functions are sintered together into a single structure.

For solving the problems mentioned above, WO 9821731 A1 discloses a low-temperature glass disposed between a surge absorber and a ceramic condenser to enhance the connection of the two materials. China Patent No. 1,858,995 discloses a varistor layer mainly composed of Zinc oxide with different additional elements to provide the material with functions of surge absorber and inductor, and then the two layers are combined by a laminating process and sintered together. KR 20020028279 shows a varistor-capacity multifunctional device based on SrCaTiO₃.

In addition, in some researches, for improving the problem of bad electrical characteristics due to mutual diffusivity during the sintering process of two materials, insulating layers with varying contents are disposed between two components.

However, although the methods mentioned above can produce components of multiple functions, the processes are relatively complicated. For instance, glass or an insulating layer with varying contents needs to be added into two materials of components to provide the components with electrical characteristics. Moreover, in such processes, two components requiring different sintering atmospheres cannot be sintered together, and thus the product cannot have good electrical characteristics.

### SUMMARY OF THE INVENTION

The present invention aims at providing a surge absorbing material for chip absorbers that has an extended range of functions and can be manufactured easily.

This technical problem is solved by a surge absorbing material according to the independent claim.

The present invention provides a surge absorbing material with dual functions. By a first-order, second-order or third-order dispersing method, conductive or semiconductive particles of micron, submicron and nanometer size are wrapped in a suitable material of a glass phase, and then sintered to have good surge absorbing characteristic. Furthermore, when the material of a glass phase is selected from materials with one of the characteristics among capacitance, inductance, voltage suppressor and thermistor, the surge absorbing material becomes a material with dual functions having one of the characteristics among capacitance, inductance, voltage suppressor and thermistor in addition to surge absorbing characteristic, and the problem of separation and ineffectiveness occurred when two materials of different characteristics are sintered together into a single structure can be solved.

When such surge absorbing material of the present invention is used in producing laminated components, the problem of cofiring different materials as a single structure is not necessarily considered any more and the laminating process is relatively simple and easy.

### BRIEF DESCRIPTION OF THE DRAWINGS

Fig. 1 is a schematic view showing microcosmic compositions of a surge absorbing material according to one preferred embodiment of the present invention.
Fig. 2 is an enlarged view of the A area in Fig. 1.
Fig. 3 is an enlarged view of the B area in Fig. 2.
Fig. 4 is a schematic view showing a laminated chip surge absorber.

### DETAILED DESCRIPTION OF THE PREFERRED EMBODIMENT

As shown from Fig. 1 to Fig. 3, the microcosmic compositions of a surge absorbing material 10 of the present invention include a high electrical resistance glass substrate 11 and micron conductive or semiconductive particles 12, submicron conductive or semiconductive particles 14 and nanometer conductive or semiconductive particles 16 uniformly distributed in the glass substrate 11.

The particle diameter of micron conductive or semiconductive particles 12 is larger than 0.1 µm, the particle diameter of submicron conductive or semiconductive particles 14 is between 0.1 to 0.01 µm, and the nanometer particle diameter of conductive or semiconductive particles 16 is smaller than 0.01 µm.

The conductive particle is selected from one or more of Pt, Pd, W, Au, Al, Ag, Ni, Cu, Fe and alloy thereof.

The semiconductive particle is selected from one of ZnO, TiO₂, SnO₂, Si, Ge, SiC, Si-Ge alloy, InSb, GaAs, InP, GaP, ZnS, ZnSe, ZnTe, SrTiO₃ and BaTiO₃.

As shown in Fig. 1, the surge absorbing material 10 of the present invention includes glass substrate 11 of 3∼60 wt% and micron conductive or semiconductive particles 12 with particle diameter more than 0.1 µm of 40∼97 wt%, based on the total weight of the surge absorbing material 10.

In addition, as shown in Fig. 2, in the microcosmic compositions of the surge absorbing material 10, second-order dispersed submicron conductive or semiconductive particles 14 are uniformly distributed in first-order dispersed micron conductive or semiconductive particles 12; as shown in Fig. 3, third-order dispersed nanometer conductive or semiconductive particles 16 are uniformly distributed in second-order dispersed submicron conductive or semiconductive particles 14.

Therefore, the microcosmic compositions of a surge absorbing material 10 include three kinds of low-resistance conductive or semiconductive particles 12, 14 and 16 with different particle diameters uniformly dispersed in the glass substrate 11, and such compositions provide the surge absorbing material 10 with the characteristic of surge absorber.

As shown in Fig. 4, when a ceramic layer 21 of a laminated chip surge absorber 20 is made by the surge absorbing material 10 according to the present invention, because the ceramic layer 21 is made of heat-resisting glass material and there are micron conductive or semiconductive particles 12 and submicron conductive or semiconductive particles 14 distributed in the microcosmic compositions of the ceramic layer 21, the laminated chip surge absorber 20 is endurable to heat generated from electrostatic shocks and surge overstresses.

Most of all, second-order dispersed submicron conductive or semiconductive particles 14 and third-order dispersed nanometer conductive or semiconductive particles 16 are further contained in the ceramic layer 21, and the particle distances of nanometer conductive or semiconductive particles 16 are so small that a tunnel effect occurs when an abnormal electrical overstress is applied. Thus, laminated chip surge absorber 20 has good electrical overstress suppressing capability and electrostatic shock resistance, as well as a good lifespan.

In sum, the surge absorbing material 10 has one of the characteristics among capacitance, inductance, voltage suppressor and thermistor in addition to surge absorbing characteristic by choosing the glass substrate 11 from one of a capacitance glass state component, an inductance glass state component, a voltage suppressor glass state component and a thermistor glass state component. In other words, the surge absorbing material 10 is a material with dual functions.

A method for producing the surge absorbing material 10 according to the preferred embodiment of the present invention includes following steps:
(1) Selecting suitable glass phase compositions to provide the glass substrate 11 of the surge absorbing material 10 with one of the characteristics among capacitance, inductance, voltage suppressor and thermistor, and using a sol-gel process to produce a solution of the glass phase composition.
   When the glass substrate 11 is the capacitance glass state composition, the glass substrate 11 can be selected from silicate glass, aluminosilicate glass, borate glass and phosphate glass with general capacitance characteristics and BaTiO₃, SrTiO₃, CaTiO₃ and TiO₂ with high dielectric constants.
   When the glass substrate 11 is the inductance glass state composition, the glass substrate 11 can be selected from a series of Ni-Zn or Ni-Cu-Zn inductance material of general inductance characteristics, or a LTCC material with high frequency inductance characteristics.
   When the glass substrate 11 is the voltage suppressor glass state composition, the glass substrate 11 can be an electrical overstress suppressing material such as BaTiO₃, PZT and PLZT.
   When the glass substrate 11 is the thermistor glass state composition, the glass substrate 11 can be a thermistor material with general thermistor characteristics such as a Mn-Ni or Mn-Co-Ni system with NTC characteristic or a V-P-Fe system with CTR characteristic.
(2) Dispersing metal or semiconductive particles of nanometer size uniformly into the glass solution in step (1).
   The nanometer particles have particle diameters smaller than 0.01 µm, and can be metal conductive particles comprising Pt, Pd, Au, Ag, Ni, Cu and so on, or semiconductive particles comprising SiC, ZnO, TiO₂, SnO₂, SrTiO₃, BaTiO₃ and so on.
(3) Dispersing conductive or semiconductive particles of submicron size uniformly into the solution having metal or semiconductive particles of nanometer dispersed therein in step (2).
(4) Dispersing conductive or semiconductive particles of micron size uniformly into the solution having submicron and nanometer metal or semiconductive particles dispersed therein in step (3).
(5) Dying and calcining the solution after step (4) at a suitable temperature (lower than 1000°C) and then milling it into a composite material to become the surge absorbing material 10 according to the preferred embodiment of the present invention.

The surge absorbing material 10 of the present invention has one of the characteristics among capacitance, inductance, voltage suppressor and thermistor in addition to surge absorbing characteristic. Thus, when producing various components from the surge absorbing material 10, which characteristic between capacitance, inductance, voltage suppressor and thermistor in addition to surge absorbing characteristic is to be provided on the component should be considered.

For instance, when the surge absorbing material 10 is a material having inductance characteristic in addition to surge absorbing characteristic, the surge absorbing material 10 may be produced as a surge absorber or a filtering component with both electromagnetic wave disturbance (EMI) preventing capability and electrostatic discharge (ESD) preventing capability. Moreover, the material of such filtering component has good surge and electrostatic absorbing capability, and the material retains original characteristics after multiple times of surge and electrostatic shocks.

## Claims

1. A surge absorbing material provided with one of the characteristics among a capacitance, an inductance, a voltage suppressor and a thermistor as well as a characteristic of a surge absorber, **characterized in that** it comprises a high electrical resistance glass substrate (11) from about 3% to about 60% by weight of the surge absorbing material; one kind of micron conductive or semiconductive particles (12) having a particle diameter larger than 0.1 µm in an amount from about 40% to about 97% by weight of the surge absorbing material, and uniformly distributed in the glass substrate, a second kind of submicron conductive or semiconductive particles (14) having a particle diameter between 0.1 to 0.01 µm and distributed in the glass substrate and in between the micron conductive or semiconductive particles; and a third kind of nanometer conductive or semiconductive particles (16) having a particle diameter smaller than 0.01 µm and distributed in the glass substrate and in between the submicron conductive or semiconductive particles, and wherein the glass substrate is selected from the group consisting of a capacitance glass state component, an inductance glass state component, a voltage suppressor glass state component and a thermistor glass state component.

2. The surge absorbing material as defined in claim 1, wherein the capacitance glass state component comprises silicate glass, aluminosilicate glass, borate glass and phosphate glass with capacitance characteristics and BaTiO₃, SrTiO₃, CaTiO₃ and TiO₂.

3. The surge absorbing material as defined in claim 1, wherein the inductance glass state component comprises a series of Ni-Zn, Ni-Cu-Zn inductance material of inductance characteristics, and a LTCC material.

4. The surge absorbing material as defined in claim 1, wherein the voltage suppressor glass state component comprises BaTiO₃, PZT and PLZT with electrical overstress suppressing characteristics.

5. The surge absorbing material as defined in claim 1, wherein the thermistor glass state component comprises a Mn-Ni, a Mn-Co-Ni system with NTC characteristic and a V-P-Fe system with CTR characteristic.

6. The surge absorbing material as defined in claim 1, wherein the conductive particle is selected from the group consisting of one or more of Pt, Pd, W, Au, Al, Ag, Ni, Cu and alloy thereof

7. The surge absorbing material as defined in claim 1, wherein the semiconductive particle is selected from the group consisting of one or more of ZnO, TiO₂, Sn02, Si, Ge, SiC, Si-Ge alloy, InSb, GaAs, InP, GaP, ZnS, ZnSe, ZnTe, SrTiO₃ and BaTiO₃.

## Patentansprüche

1. Material zur Absorption von elektrischen Störimpulsen mit einer der Eigenschaften aus Kapazität, Induktivität, Spannungsunterdrücker und Thermistor sowie der Eigenschaft eines Überspannungsschutzes, **dadurch gekennzeichnet, dass** dieses umfasst ein Glassubstrat (11) mit hohem elektrischen Widerstand aus etwa 3 bis etwa 60 Gewichtsprozent des Materials zur Absorption von elektrischen Störimpulsen; eine Art von leitenden oder halbleitenden Mikropartikeln (12) mit einem Partikeldurchmesser größer als 0,1 µm in einer Menge von etwa 40 bis etwa 97 Gewichtsprozent des Materials zur Absorption von elektrischen Störimpulsen, welche gleichmäßig in dem Glassubstrat verteilt sind, eine zweite Art von leitenden oder halbleitenden Submikropartikeln (14) mit einem Partikeldurchmesser zwischen 0,1 und 0,01 µm, welche in dem Glassubstrat und zwischen den leitenden oder halbleitenden Mikropartikeln verteilt sind; und eine dritte Art von leitenden oder halbleitenden Nanopartikeln (16) mit einem Partikeldurchmesser kleiner als 0,01 µm, welche in dem Glassubstrat und zwischen den leitenden oder halbleitenden Submikropartikeln verteilt sind, und wobei das Glassubstrat aus der Gruppe gewählt ist, die aus einer Kapazitätskomponente im Glaszustand, einer Induktivitätskomponente im Glaszustand, einer Spannungsunterdrückungskomponente im Glaszustand und einer Thermistorkomponente im Glaszustand besteht.

2. Material zur Absorption von elektrischen Störimpulsen nach Anspruch 1, bei dem die Kapazitätskomponente im Glaszustand Silikatglas, Aluminosilikatglas, Boratglas und Phosphatglas mit kapazitiven Eigenschaften und BaTiO₃, SrTiO₃, CaTiO₃ und TiO₂ umfasst.

3. Material zur Absorption von elektrischen Störimpulsen nach Anspruch 1, bei dem die Induktivitätskomponente im Glaszustand eine Folge von Ni-Zn, Ni-Cu-Zn-Induktanzmaterial mit induktiven Eigenschaften und ein LTCC-Material umfasst.

4. Material zur Absorption von elektrischen Störimpulsen nach Anspruch 1, bei dem die Spannungsunterdrückungskomponente im Glaszustand BaTiO₃, PZT und PLZT mit elektrischen Überlastungsschutzeigenschaften umfasst.

5. Material zur Absorption von elektrischen Störimpulsen nach Anspruch 1, bei dem die Thermistorkomponente im Glaszustand ein Mn-Ni, ein Mn-Co-Ni-System mit NTC-Verhalten und ein V-P-Fe-System mit CTR-Eigenschaften umfasst.

6. Material zur Absorption von elektrischen Störimpulsen nach Anspruch 1, bei dem das leitende Partikel aus der Gruppe gewählt ist, die aus einem oder mehreren aus Pt, Pd, W, Au, Al, Ag, Ni, Cu und Legierungen daraus besteht.

7. Material zur Absorption von elektrischen Störimpulsen nach Anspruch 1, bei dem das halbleitende Partikel aus der Gruppe gewählt ist, die aus einem oder mehreren aus ZnO, TiO₂, SnO₂, Si, Ge, SiC, Si-Ge-Legierung, InSb, GaAs, InP, GaP, ZnS, ZnSe, ZnTe, SrTiO₃ und BaTiO₃ besteht.

## Revendications

1. Matériau absorbant des impulsions parasites pourvu d'une des caractéristiques parmi la capacité, l'inductance, un suppresseur de tension et une thermistance aussi bien qu'une caractéristique d'absorption d'impulsions parasites, **caractérisé en ce qu'**il comprend un substrat en verre à résistance électrique élevée (11) d'environ 3% à environ 60% par poids du matériau absorbant des impulsions parasites; un type de particules conductrices ou semiconductrices (12) de la taille d'un micron ayant un diamètre de particule supérieur à 0,1 µm en une quantité d'environ 40% à environ 97% en poids du matériau absorbant des impulsions parasites et distribuées uniformément dans le substrat en verre, un second type de particules conductrices ou semiconductrices inférieures au micron (14) ayant un diamètre de particules entre 0,1 et 0,01 µm et distribuées dans le substrat en verre et entre les particules conductrices ou semiconductrices de la taille d'un micron; et un troisième type de particules conductrices ou semiconductrices de la taille d'un nanomètre (16) ayant un diamètre de particules inférieur à 0,01 µm et distribuées dans le substrat en verre et entre les particules conductrices ou semiconductrices inférieures au micron et le substrat en verre étant sélectionné dans le groupe consistant en un composant de capacitance à l'état de verre, un composant d'inductance à l'état de verre, un composant suppresseur de tension à l'état de verre et un composant de thermistance à l'état de verre.

2. Matériau absorbant des impulsions parasites selon la revendication 1, le composant de capacitance à l'état de verre comprenant du verre au silicate, du verre à l'aluminosilicate, du verre au borate et du verre au phosphate avec des caractéristiques de capacitance et du BaTiO₃, du SrTiO₃, du CaTi O₃ et du TiO₂.

3. Matériau absorbant des impulsions parasites selon la revendication 1, le composant d'inductance à l'état de verre comprenant une série de matériau d'inductance au Ni-Zn, au Ni-Cu-Zn avec caractéristiques d'inductance et un matériau CCBT.

4. Matériau absorbant des impulsions parasites selon la revendication 1, le composant suppresseur de tension à l'état de verre comprenant du BaTiO₃, du PZT et du PLZT avec des caractéristiques de suppression de surtension électrique.

5. Matériau absorbant des impulsions parasites selon la revendication 1, le composant de thermistance à l'état de verre comprenant un système au Mn-Ni, au Mn-Co-Ni avec des caractéristiques CTN et un système de V-P-Fe avec caractéristique CTR.

6. Matériau absorbant des impulsions parasites selon la revendication 1, la particule conductrice étant sélectionnée dans le groupe consistant en un ou plusieurs des éléments Pt, Pd, W, Au, Al, Ag, Ni, Cu et les alliages de ceux-ci.

7. Matériau absorbant des impulsions parasites selon la revendication 1, la particule semiconductrice étant sélectionnée dans le groupe consistant en un ou plusieurs des éléments ZnO, TiO₂, SnO₂, Si, Ge, SiC, alliage de Si-Ge, InSb, GaAs, InP, GaP, ZnS, ZnSe, ZnTe, SrTiO₃ et BaTiO₃.
